

## UNITED STATES PATENT OFFICE

FRANK AMBROSIO, OF BROOKLYN, NEW YORK, ASSIGNOR OF ONE-THIRD TO HARRY GRASSER, OF LONG BEACH, NEW YORK

## PLASTERING

No Drawing.

Application filed January 16, 1931. Serial No. 509,271.

This invention relates to plaster and has for its object the provision of certain improvements in plastering. More particularly, the invention aims to provide an improved method of plastering which substantially shortens the time within which walls may be completely plastered and ready for decoration (if any) by papering, painting and the like. The invention further aims to provide an improved method of plastering which permits the application of the finishing layer of plaster directly after the foundation layer of plaster and while the latter is still wet. Another object of the invention is the provision, as a new article of commerce, of a novel plaster composition, particularly adapted for finishing purposes.

In applying plaster upon such foundations as laths and the like, it has heretofore been the common practice to first apply directly on the laths (or other appropriate foundation) a relatively thick layer of coarse plaster, and when this has set and dried to apply a thinner layer or coat of fine finishing plaster. The first layer of coarse plaster has commonly been made up of about 1 part of neat gypsum plaster and about 3 parts of sand with sufficient water to form a mass of the desired consistency. Commercial neat gypsum plaster, as it ordinarily appears on the market, contains about 85% of calcined gypsum and the remaining 15% is made up of hydrated lime, clay, asbestos, fibre and retarder. About 3 to 4 days are usually required for the drying and hardening of this first layer of coarse plaster. The fine or finishing coat of plaster is commonly made up of about 5 parts of hydrated finishing lime and about 1 part of plaster of Paris with sufficient water to form a mixture of the desired consistency. This finishing coat cannot be applied to the layer of coarse plaster until the latter has dried and hardened, and about 3 days are required for the drying of the finishing coat of plaster. It is thus a week, and frequently much longer, before a plastered wall is completed and ready for decoration by papering, painting or the like.

The present invention involves the application on an appropriate foundation of two

layers or coats of plaster, the second layer or coat being applied immediately after the first layer or coat and before the latter has set or dried to any substantial amount. The first layer of plaster applied directly on the foundation is a relatively strong and quick setting plaster, as compared with the heretofore common first or coarse layer of plaster. The second layer of plaster, applied directly on the first layer while the latter is still wet, is a stronger and more rapid setting plaster than the first layer. The first layer of plaster may be considerably thinner than the heretofore customary first or coarse layer of plaster and the second or finishing layer of plaster may be somewhat thinner than the heretofore customary finishing coat of plaster.

Each of the plaster layers of the invention consists in large part of gypsum plaster, and the second or finishing layer contains in addition a substantial amount of plaster of Paris; the combined amount of gypsum plaster and plaster of Paris being preferably about 60 to 75% of the total plaster composition.

The first layer of plaster may advantageously be made up of gypsum plaster and sand with the gypsum plaster in excess of the sand. It is now my preferred practice to make up the plaster for this first layer of approximately 2 parts (say 60 to 75%) of neat gypsum plaster and 1 part of sand.

The plaster for the finishing coat or layer preferably contains hydrated finishing lime and an inert strengthening material, in addition to gypsum plaster and plaster of Paris. Very satisfactory results are obtained with a plaster containing approximately equal parts of gypsum plaster and plaster of Paris with the amount of each in excess of the amount of lime and also in excess of the amount of inert material, when the latter is present. It is now my preferred practice to make up the finishing plaster of approximately 2 parts of neat gypsum plaster, 2 parts of plaster of Paris, 1 part of hydrated finishing lime and 1 part of marble dust or other appropriate inert strengthening material.

In practicing the invention, the first layer of plaster is applied directly on the laths or

- other appropriate foundation. Because of its relatively quick setting property the plaster should be applied as expeditiously as practicable. The second or finishing layer of 5 plaster is applied directly on the wet first layer of plaster and must be worked rapidly since in its preferred form it sets or hardens in from one to two hours. The finishing layer of plaster is well adapted to produce the 10 prevailing popular art-craft effects, and it is accordingly my preferred practice in applying the finishing coat to rapidly work it so as to produce such effects before the plaster begins to take on a permanent set. 15 One of the characteristic features of novelty of the present invention is the ability to apply the finishing layer of plaster to the first layer of plaster while the latter is wet. As a matter of fact, my experience in practicing the invention indicates that the first 20 layer of plaster should be wet when the finishing layer is applied thereto, since otherwise the first layer of plaster so rapidly absorbs moisture from the finishing layer as to prevent proper working thereof. The rapid 25 setting or hardening of the finishing layer appears also to prevent cracking of the first layer. In other words, the first layer does not completely dry or harden for some time 30 after the finishing layer has set and hardened, and the finishing layer thus appears to provide a hard protective coating on the first layer which effectively prevents cracking or rupture of the latter. It thus becomes possible 35 by the practice of the invention to completely form a finished plastered wall in about one day's time, the wall being then ready for the application of any desired decorative effects. 40 I claim:  
1. The improvement in plastering which comprises applying to an appropriate foundation a layer of a relatively strong and quick-setting gypsum plaster, and applying 45 to said layer of gypsum plaster while still wet a layer of a stronger and more rapid setting plaster.  
2. The improvement in plastering which 50 comprises applying to an appropriate foundation a layer of plaster containing gypsum and sand with the gypsum in excess, and applying to said layer of plaster while still wet a layer of a relatively stronger and more rapid setting plaster.  
3. The improvement in plastering which 55 comprises applying to an appropriate foundation a layer of a relatively strong and quick-setting gypsum plaster, and applying to said layer of plaster while still wet a layer of a relatively stronger and more rapid setting plaster containing approximately equal amounts of gypsum plaster and plaster of Paris.  
4. The improvement in plastering which 60 comprises applying to an appropriate foun-

dation a layer of a relatively strong and quick-setting plaster, and applying to said layer of plaster while still wet a layer of a relatively stronger and more rapid setting plaster containing from 60 to 75% of gypsum plaster and plaster of Paris in approximately equal amounts. 70

5. The improvement in plastering which comprises applying to an appropriate foundation a layer of plaster containing gypsum and sand with the gypsum in excess, and applying to said layer of plaster while still wet another layer of plaster containing gypsum plaster, plaster of Paris and hydrated finishing lime with the gypsum and plaster of Paris each in excess of the lime. 75

6. The improvement in plastering which comprises applying to an appropriate foundation a layer of a relatively strong and quick-setting gypsum plaster, and applying to said layer of gypsum plaster while still wet another layer of plaster containing gypsum plaster, plaster of Paris and hydrated finishing lime with the gypsum and plaster of Paris each in excess of the lime. 80

7. The improvement in plastering which comprises applying to an appropriate foundation a layer of a relatively quick-setting gypsum plaster, and applying to said layer of gypsum plaster while still wet another layer of a relatively more rapid setting gypsum plaster. 85

In testimony whereof I affix my signature.  
FRANK AMBROSIO.

700

105

110

115

120

125

130